

## UNITED STATES PATENT OFFICE.

HYMAN STEIN AND WILLIAM E. AUSTIN, OF NEW YORK, AND IRVING LIEBOWITZ, OF BROOKLYN, NEW YORK, ASSIGNEES TO STEIN FUR DYEING CO., INC., OF NEW YORK, N. Y., A CORPORATION OF NEW YORK.

FELT AND FELT MATERIAL AND ARTICLES, SUCH AS HATS AND HAT BODIES MADE OF THE SAME.

No Drawing. Application filed February 10, 1925. Serial No. 8,307.

Our present invention relates to animal fibers, particularly such fibers in a condition well suited for felting operations, and to the felted products themselves, and aims to devise animal fibers of the general character specified above which are in a condition remarkably well suited for subsequent felting operations and very well adapted to produce felted products of a high degree of quality. In particular, our present invention relates to a readily feltable animal fiber which, while retaining its natural strength to a very large degree, is not only readily feltable but is rendered, either before, during or after the "carrotting" or equivalent operation, of a light color, so as to enable the same, either simultaneously with or after the bleaching operation, to be dyed a light or other suitable color. My invention relates also to the resulting mass of feltable fibers and to the felted fabric itself, as well as the partially or completely shaped felted bodies, such as blocked felt hat bodies incorporating the feltable fibers or felted fabrics of the present invention.

In the accompanying specification we shall describe illustrative embodiments of the products of the present invention. It is, however, to be clearly understood that our invention is not limited to the specific embodiments thereof herein described for purposes of illustration merely. It is further to be understood that the processes for making the products of the present invention, as herein described in order to make the present invention clear and the description of the same such as to enable persons skilled in the art to practice the invention, are claimed in a copending application of ours filed of even date herewith and entitled "Methods of fabricating felts and felt materials" Serial No. 8,306.

Before describing in detail the aforesaid illustrative embodiments of the present invention, it may be desirable briefly to point out certain disadvantages of the prior art so far as the same relates to the field of the present invention. Hitherto it has been proposed, for example, to "carrot" animal fibers, such as fur skins and the like or the hair of such skins, to render the same suitable for felting operations, by treating such skins or

the hair of the same with an acid solution of nitrate of mercury. This treatment, if used by itself for the entire "carrotting" operation, tends to weaken and otherwise hurt the hairs or equivalent fibers.

Furthermore, where it is desired to obtain a light colored mass of feltable hairs or other animal fibers, if the hair is bleached first, the bleaching operation generally tends to weaken the hair to such an extent that the subsequent "carrotting" operation, tending further to weaken the hair, would tend often to render the same quite unfit for the subsequent felting operation. It has, therefore, not been feasible to make a light colored mechanically desirable feltable fiber from a dark colored skin by the usual bleaching and "carrotting" operations.

On the other hand, if the hair or equivalent animal fibers are first "carroted", as by means of the treatment with the acid solution of nitrate of mercury referred to above, this treatment would tend to render the subsequent bleaching operation imperfect and otherwise quite unsatisfactory. In any event, both the "carrotting" and the bleaching operations as hitherto conducted, in whatever order they have been carried out, would both singly and conjointly tend to considerably weaken and otherwise impair the structure and appearance, as well as the felting qualities, of the fur, hair or other fibers to which the treatments of the prior art might be applied.

We have discovered that feltable fibers and felted masses of such fibers, as well as the felted fabrics themselves and the partially or completely shaped bodies, such as hat bodies, incorporating such feltable fibers or fabrics, may be made in accordance with the methods described and claimed in our copending application filed of even date herewith and referred to above. In practicing the methods of our aforesaid application in the production of the products of the present invention, we take first any suitable fur skin or the hair of such skin, or any other suitable animal fiber which it is desired to convert into a feltable fiber. Preferably we treat a fiber which is dark and which we desire to bleach into a light colored readily feltable fiber. For example,

we may take rabbit skins of a dark color and treat the same with great success in accordance with the principles of the present invention.

5 It may here be stated that the products of the present invention may be obtained with almost equal success either from the fur skin itself, such as the dark or other colored rabbit skins referred to, or from the hair obtained from such skins. In fabricating the products of the present invention, neither the fur skins nor the hair derived from the same need first be washed or "killed" in an alkaline solution, such as a solution of sodium carbonate. However, in some instances, this washing operation, which ordinarily requires from about two to about three hours, may be employed, although we prefer to dispense with the same in most instances.

10 20 We now treat the fur skins or the hair of the same, referred to above, preferably the dark or other colored rabbit skins or hair from such skins, with a suitable "carrotting" agent, preferably a metallic "carrotting" agent, but preferably only to the point of partial completion of the "carrotting" step. For example, we may treat the fur skins or other animal fibers in the fabrication of the products of the present invention with nitrate of mercury, obtained, for example, by the solution of metallic mercury in nitric acid, thus obtaining an acid solution of nitrate of mercury. This treatment is preferably continued only to the point of partial completion of the "carrotting" operation, as by using only one-half, or only two-thirds or three-fourths, or any suitable amount of the acid solution of the nitrate of mercury or equivalent metallic or other "carrotting" agent, short of the amount which would be required for the completion of the "carrotting" operation. This is very desirable, since the subsequent bleaching operation serves, at the same time, to complete the "carrotting" operation, all of which is done in the fabrication of the products of the present invention without destruction of the hair or other animal fibers and without in any way impairing their ultimate felting qualities. In fact, the felting qualities of animal fibers treated in the fabrication of the products of the present invention are superior to those of ordinary fibers treated in accordance with the methods hitherto employed for this purpose.

15 25 30 35 40 45 50 55 60 65 70 75 80 85 90 95 100 105 110 115 120 125 We now treat the partially "carroted" fibers, prior to the subsequent bleaching and completion of the "carrotting" process, with a protective agent, generally a reducing compound, preferably of mineral origin, such as a ferrous compound, for example, ferrous sulphate. In some way, the reasons for which are at present not understood by us, such protective agent, while permitting the

bleaching or decolorizing action to proceed 65 under the action of the bleaching agent with remarkable rapidity, protects the leather of the fur skin and the hair of the same from any destructive or weakening effect of the bleaching agent.

70 75 80 85 90 95 100 105 110 115 120 125 For instance, decolorizing or bleaching of fur skins, hair or the like, in the production of the products of the present invention, takes place under the action of a bleaching agent such as hydrogen peroxide, for example, within a short time, as from about one to about four hours. This is contrasted with the twenty-four to seventy-two hours hitherto required for bleaching fur skins by the methods hitherto commonly employed. At the same time the leather and hair of the skins and the fibers of the hair or other animal fibers bleached in the fabrication of the products of the present invention will be found to be in fine condition, with their strength, texture and lustre substantially unimpaired. At the same time, we have discovered that the "carrotting" operation is completed by what we have thus far termed the "bleaching" operation. It appears that the hydrogen peroxide or equivalent bleaching agent acts as a non-metallic "carrotting" agent to complete the "carrotting" operation only partially completed by the acid solution of nitrate of mercury or equivalent metallic "carrotting" agent.

100 105 110 115 120 125 While we do not wish to be limited to any particular theory or explanation as to why this remarkable, unexpected and commercially valuable result is obtained, our present explanation is that the presence on or in the fibers of the fur skins or the like of the mineral reducing agent or its equivalent, the effectiveness of which appears not to be diminished by the presence of the nitrate of mercury or other metallic "carrotting" agent, prevents too violent an action of the hydrogen peroxide or equivalent bleaching agent. At the same time, the hydrogen peroxide or equivalent bleaching agent acts to complete the "carrotting" operation and the ultimate product is a fiber light in color and remarkably well adapted for subsequent felting operations. In fact, the presence of the metallic protective agent, such as the ferrous compound referred to, or its equivalent, especially in the presence of the nitrate of mercury or equivalent metallic compound "carrotting" agent, not only protects the leather and the hair of the fur skins or other animal fibers from destructive or weakening action, but at the same time actually accelerates the desired decolorizing or bleaching action and the completion of the "carrotting" operation, so that the combined bleaching and "carrotting" operation take only from about one to about four hours, instead of the twenty-four to seventy-two

hours hitherto required for the imperfect or even destructive bleaching methods as hitherto practiced.

Since the protective agent and bleaching accelerator, in the fabrication of the products of the present invention, generally comprises a reducing agent or compound, preferably of mineral origin, such as a ferrous compound, for example, ferrous sulphate, which would tend to be oxidized more or less readily on exposure to the air, we prefer to add to the protective agent preferably before the same is applied to the fur skin or the like, prior to the bleaching and "carrotting" operation, a stabilizing agent. The purpose of the stabilizing agent is to stabilize the protective agent and to prevent too rapid oxidation or deterioration of the same. Where, as is preferred, ferrous sulphate is used for the protective agent, we prefer to use for the stabilizing agent ammonium chloride. The fur skins or the like, after having been treated with a solution of the protective compound which may or may not contain therein the stabilizing agent, are thereafter subjected to the combined bleaching and "carrotting" operation, after which they may be dyed in any of the light or other shades such as can at the present time be produced only by dyeing natural white or other light colored skins or other animal fibers.

The following is a specific example of one mode of applying the method in the fabrication of the products of the present invention it being understood, however, that the following description is given merely by way of illustration and that the process is not limited to the specific details of the following illustrative example:

The dark colored rabbit skins, preferably without being first washed or "killed" in an alkaline solution, such as a solution of sodium carbonate, which washing operation ordinarily requires from about two to about three hours, are immersed in an acid solution of nitrate of mercury in an amount sufficient only partially to "carrot" such skins or like animal fibers. For example, only one-half, or even as much as two-thirds or three-fourths, of the usual amount of acid solution of nitrate of mercury is employed so that the "carrotting" operation at this stage is only partially completed.

The partially "carroted" skins or other animal fibers are then rinsed and thoroughly hydro-extracted. The skins are then immersed in a solution of the protective agent, such as in a solution of ferrous sulphate, and there allowed to remain overnight. While the strength of the ferrous sulphate solution or its equivalent may vary within considerable limits, we prefer to use an aqueous solution of ferrous sulphate of a strength of from about 0.5 to about 5.0 per cent of the solid

crystallized ferrous sulphate, by weight. Such a solution may or may not contain the stabilizing agent. If a stabilizing agent, such as ammonium chloride, is used, we prefer to use it in an amount approximately proportionate to the amount of ferrous sulphate used and equalling from about 0.5 to about 5.0 per cent of ammonium chloride, by weight.

The fur skins or the like, after having been soaked for from about 8 to about 12 hours in the solution of the protective agent, with or without the addition of the stabilizing agent, are then rinsed and hydro-extracted. The treatment apparently impregnates or fills the voids and interstices of the fibers with the solution of protective agent. The fur skins thus treated are now immersed in a solution of hydrogen peroxide or equivalent bleaching agent. However, in place of hydrogen peroxide, we may use other bleaching agents, particularly sodium peroxide or sodium perborate, which yield hydrogen peroxide in solution in the presence of certain liberating agents, generally of an acid character. The amount of hydrogen peroxide used may vary from about five (5.0) to about one hundred (100.0) per cent by volume of a three (3.0) per cent solution of hydrogen peroxide. We prefer that the temperature at which the bleaching or decolorizing operation is carried out shall be between 60° and 100° F.

The skins or hair are subjected to the action of the bleaching and "carrotting" agent until they have been sufficiently decolorized. The bleached and now completely "carroted" skins are then rinsed and can, if desired, be dyed directly in accordance with any of the well-known or desirable processes employed for dyeing furs or the like. We may, however, subject the bleached or decolorized skins or hair to the usual dyeing operations of washing and mordanting, and then dyeing the washed and mordanted skins or hair in accordance with the practice hitherto generally employed for dyeing furs and hair.

It may here be stated that a metallic salt or salts may be added to the solution of the protective agent, with or without the stabilizing agent, provided such metallic salt or salts are compatible with the ferrous sulphate of equivalent protective agent. In such a case, the combined decolorizing and "carrotting" process proceeds in exactly the same way as before, while the additional salt or salts may act as a mordant for the subsequent dyeing process where a mordant is desired or needed for this purpose. It may here also be stated that while, in accordance with our experience up to the present time, the foregoing process may be successfully applied to all dark colored furs, the concentration of the reagents employed and the

methods of subjecting the fur skins or the like to the various partial "carrotting", protective, and combined bleaching and "carrotting" operations, as well as the subsequent 5 mordanting and dyeing operations, will depend very largely upon the nature of the skins of other animal fibers being treated, the factors of temperatures, concentrations, 10 lengths of time of treatment, and the like, for any particular kind of animal fiber or the like, being readily determined by trial and experiment.

It may here be stated that in addition to the mineral protective agent, such as the 15 ferrous sulphate, with or without the addition of the stabilizing agent, the solution for giving the fur skins or the like their protective treatment for the subsequent combined bleaching and "carrotting" operation 20 may contain other compatible metal salts, as well as suitable protective colloids, such as glue, gelatin, or the like, generally in relatively small amounts. It may here also be stated that the methods described above may be applied with almost equal success in the treatment of skins which have already been dyed, either a dark or a light color, and whether satisfactorily or not, but preferably skins which have been dyed by the use of a mordant 25 consisting of a ferrous compound, such as ferrous sulphate, or an equivalent substance, thus producing from the previously dyed skins and hair the superior products described above.

35 It may here be stated that under certain conditions the combined bleaching and "carrotting" operation by means of a non-metallic "carrotting" agent may be carried out first, after which the "carrotting" operation may 40 be completed by regulating the amount and length of time of treatment with the acid solution of nitrate of mercury or its equivalent. It may here also be stated that the bleaching operation may be carried out with 45 complete success on fibers or even felts already completely "carroted" by treatment with an acid solution of nitrate of mercury or equivalent reagent. In fact, the bleaching operation may be carried out with remarkable 50 success on shaped felted bodies such as hat bodies, after the "carrotting" operation has been completed. Or else such fibers, masses of felt, or shaped felted bodies 55 may first be bleached and partially "carroted" and thereafter "carroted" to completion as already indicated above.

The products of the present invention, particularly as fabricated by the aforesaid 60 illustrative embodiments of the method more fully described and claimed in our copending application filed of even date herewith and already referred to above, are characterized by the remarkable felting properties of such fibers, and the strength 65 of the felted fabrics and felt bodies made

from such fibers and fabrics. At the same time, even where a dark colored rabbit or other skin or hair obtained from the same is used as the source of the hair or other animal fibers from which the products of the present invention are obtained, we may obtain as an ultimate product a light colored feltable fiber or felted mass, or felted fabric or felt bodies, otherwise obtainable only from the comparatively expensive natural 75 white or light colored skins or hair obtained from the same. The products of the present invention are characterized further by their comparative cheapness, which gives the same a very wide demand and a very profitable market. Other advantages and 80 priorities of the products of the present invention will readily occur to those skilled in the art to which the same relates.

What we claim as our invention is:

1. A feltable animal fibre impregnated with mercurial and iron compounds.
2. A feltable animal fibre incorporating a carrotting agent and a protective compound to protect the fibre from excessive chemical 90 action thereon by the bleaching agent.
3. A feltable animal fibre incorporating a metallic salt carrotting agent and a protective compound to protect the fibre from excessive chemical action thereon by the bleaching agent.
4. A feltable animal fibre incorporating a mercurial carrotting agent and a protective compound to protect the fibre from excessive chemical action thereon by the bleaching 100 agent.
5. A feltable animal fibre incorporating a metallic salt carrotting agent and a metallic salt protective compound to protect the fibre from excessive chemical action thereon by the bleaching agent.
6. A feltable animal fibre incorporating a mercurial carrotting agent and a metallic salt protective compound to protect the fibre from excessive chemical action thereon by the bleaching agent.
7. A feltable animal fibre incorporating a carrotting agent and a metallic salt protective compound to protect the fibre from excessive chemical action thereon by the bleaching agent.
8. A feltable animal fibre incorporating a mercurial carrotting agent and a metallic salt protective compound in the form of a compound of iron to protect the fibre from excessive chemical action thereon by the bleaching agent.
9. A feltable animal fibre incorporating a metallic salt carrotting agent and a metallic salt protective compound in the form of a compound of iron to protect the fibre from excessive chemical action thereon by the bleaching agent.
10. A feltable animal fibre incorporating a carrotting agent and a metallic salt pro-

tective compound in the form of a compound of iron to protect the fibre from excessive chemical action thereon by the bleaching agent.

5 11. A felted fabric comprising an inter-  
laced and interfelted mass of bleached ani-  
mal fibres treated with a carotting agent  
and a protective and accelerating compound,  
said protective and accelerating compound  
10 having served to protect the fibres of said  
fabric from excessive chemical action there-  
on by the bleaching agent.

12. A felted fabric comprising an interlaced and interfelted mass of bleached animal fibres treated with a metallic salt-carboning agent and a protective and accelerating compound, said protective and accelerating compound having served to protect the fibres of said fabric from excessive chemical action thereon by the bleaching agent.

13. A felted fabric comprising an interlaced and interfelted mass of bleached animal fibres treated with a mercurial carotting agent, and a protective and accelerating compound, said protective and accelerating compound having served to protect the fibres of said fabric from excessive chemical action thereon by the bleaching agent.

14. A felted fabric comprising an inter-laced and interfelted mass of bleached animal fibres treated with a mercurial carotting agent and a metallic salt protective and accelerating compound, said protective and accelerating compound having served to protect the fibres of said fabric from excessive chemical action thereon by the bleaching agent.

15. A felted fabric comprising an interlaced and interfelted mass of bleached animal fibres treated with a metallic salt carotting agent and a metallic salt protective and accelerating compound, said protective and accelerating compound having served to protect the fibres of said fabric from excessive chemical action thereon by the bleaching agent.

16. A felted fabric comprising an interlaced and interfelted mass of bleached animal fibres treated with a carotting agent and a metallic salt protective and accelerating compound, said protective and accelerating compound having served to protect the fibres of said fabric from excessive chemical action thereon by the bleaching agent.

55 17. A felted fabric comprising an inter-  
laced and interfelted mass of animal fibres  
treated with a carotting agent and a metal-  
lic salt protective and accelerating compound  
and bleached with hydrogen peroxide, said  
protective and accelerating compound hav-  
ing served to protect the fibres of said fabric  
from excessive chemical action thereon by  
said hydrogen peroxide.

18. A felted fabric comprising an interlaced and interfelted mass of animal fibres treated with a metallic carotting agent and a

metallic salt protective and accelerating compound and bleached with hydrogen peroxide, said protective and accelerating compound having served to protect the fibres of said fabric from excessive chemical action thereon by said hydrogen peroxide. 70

19. A felted fabric comprising an interlaced and interfelted mass of animal fibres treated with a mercurial carotting agent and a metallic salt protective and accelerating compound and bleached with hydrogen peroxide, said protective and accelerating compound having served to protect the fibres of said fabric from excessive chemical action thereon by said hydrogen peroxide. 75 80

20. A felted fabric comprising an interlaced and interfelted mass of animal fibres treated with a mercurial carotting agent and a protective and accelerating compound and bleached with hydrogen peroxide, said protective and accelerating compound having served to protect the fibres of said fabric from excessive chemical action thereon by said hydrogen peroxide. 85

21. A felted fabric comprising an interlaced and interfelted mass of animal fibres treated with a metallic carotting agent and a metallic salt protective and accelerating compound in the form of a compound of iron and bleached with hydrogen peroxide, said protective and accelerating compound having served to protect the fibres of said fabric from excessive chemical action thereon by said hydrogen peroxide. 90 95

22. A felted fabric comprising an interlaced and interfelted mass of animal fibres treated with a carotting agent and a metallic salt protective and accelerating compound in the form of a compound of iron and bleached with hydrogen peroxide, said protective and accelerating compound having served to protect the fibres of said fabric from excessive chemical action thereon by said hydrogen peroxide. 100 103

23. A felted fabric comprising an interlaced and interfelted mass of animal fibres treated with a mercurial carotting agent and a protective and accelerating compound and bleached with hydrogen peroxide, said protective and accelerating compound having served to protect the fibres of said fabric from excessive chemical action thereon by said hydrogen peroxide. 110 115

24. A felted fabric comprising an interlaced and interfelted mass of animal fibres 120 treated with a mercurial carotting agent and a metallic salt protective and accelerating compound in the form of a compound of iron and bleached with hydrogen peroxide, said protective and accelerating compound having 125 served to protect the fibres of said fabric from excessive chemical action thereon by said hydrogen peroxide.

25. A felted fabric comprising an interlaced and interfelted mass of animal fibres 130

treated with a metallic salt carotting agent and a metallic salt protective and accelerating compound and bleached with hydrogen peroxide, said protective and accelerating compound having served to protect the fibres of said fabric from excessive chemical action thereon by said hydrogen peroxide.

26. A bleached feltable animal fibre im-

pregnated with mercurial and iron compounds. <sup>10</sup>

In testimony whereof, we have signed our names to this specification this 29th day of January, 1925.

HYMAN STEIN.

IRVING LIEBOWITZ.

WILLIAM E. AUSTIN.